

Feb. 22, 1944.

G. VAN NIMWEGEN

2,342,313

ABRASIVE ARTICLE

Filed Sept. 6, 1941

*Fig. 1*



*Fig. 2.*



INVENTOR.  
GARRET VAN NIMWEGEN

*R. C. Barnes*  
ATTORNEY.

## UNITED STATES PATENT OFFICE

2,342,313

## ABRASIVE ARTICLE

Garret Van Nimwegen, Niagara Falls, N. Y., assignor to The Carborundum Company, Niagara Falls, N. Y., a corporation of Delaware

Application September 6, 1941, Serial No. 409,812

11 Claims. (Cl. 51—298)

This invention relates to bonded abrasive articles, and more particularly to abrasive articles in which the abrasive portions of the articles are supported by metallic or other rigid means, such as metal backing plates or side plates secured to the flat faces of abrasive sections, metal or other rigid rings fastened to the back or inner surface of annular-shaped abrasive articles, or spindles attached to various abrasive shapes for the purpose of mounting on grinding apparatus. Especially the invention concerns the means of securing these supporting plates, rings, spindles and the like to the abrasive portions of the articles.

This application is a continuation-in-part of application Serial No. 303,279 filed November 7, 1939.

The invention has been found particularly applicable to the making of disc-shaped grinding wheels adapted to be mounted for grinding with the flat side face of the wheel. Therefore, for the purposes of simplicity and clarity, the invention will be described mostly as it applies to the making of such disc wheels.

It has been found in the past that many heavy duty grinding operations can be performed most efficiently by presenting the work to the flat face of a disc-shaped grinding wheel. However, this type of grinding operation subjects the wheel to extremely high stresses and strains, particularly that part of the wheel where the abrasive section is joined to the backing plate or mounting. As a result, failure of the wheel frequently occurs because of weakness of the wheel at the joint between the backing plate and the abrasive section. Wheels in which the backing is attached to the abrasive portion by means of a layer of vulcanized rubber are subject to failure before the useful life of the abrasive has been obtained because of the deterioration of the rubber under the heat of grinding. Further failures are caused in wet grinding by attack on the rubber layer by cooling agents such as kerosene, oils and other hydrocarbon cooling agents.

An object of the present invention is to provide an improved means of securing bonded abrasive sections to rigid, metal supporting or mounting plates, rings, spindles and the like.

Another object of the present invention is to provide an improved bonded abrasive article in which the bonded abrasive body of the article is strongly and firmly secured to a backing plate, ring, spindle or the like.

Another object of the invention is to provide a backed grinding wheel or disc which will be

sufficiently heat resistant to stand up under the heat of heavy duty grinding operations for the normal life of the abrasive portion of the wheel, which can be operated at high grinding speeds, which will be resistant to kerosene, oils, caustic, hydrocarbons and other cooling agents used in wet grinding and can therefore be used for both wet and dry grinding, and which will possess a high energy absorption power and a high rate of damping of vibrations set up in grinding.

In accordance with the present invention, an abrasive article is provided with a metallic supporting or mounting means secured to the bonded abrasive section by means of an intermediate bonding layer (herein referred to as a tie bond) which is strongly adherent to both the metal supporting means and to the bonded abrasive section, and which retains the greater part of its strength in the presence of cooling agents and extreme temperatures involved in grinding operations. A specific application is the attachment of rigid, metal backing plates to the backs of disc-shaped grinding wheels for use in heavy duty side grinding operations. A tie bond material which has been discovered to be highly effective is polychloroprene which has been suitably compounded. Another highly satisfactory tie bond material is the copolymer of butadiene (divinyl) with acrylonitrile. Among other vulcanizable synthetic elastic materials which are satisfactory are polyvinylchloride, butadiene (divinyl) polymers, polyethylene sulphide, polybromoprene, copolymers of butadiene (divinyl) with styrene, copolymers of butadiene (divinyl) with methyl methacrylate, copolymers of butadiene (divinyl) with isobutylene, copolymers of butadiene (divinyl) with coumarone or indene, copolymers of butadiene (divinyl) with vinylidene chloride, copolymers of butadiene with chloromethacrylic ester, copolymers of chloroprene with acrylonitrile, copolymers of chloroprene with styrene, copolymers of chloroprene with methyl methacrylate, and other copolymers of butadiene or halogen-substituted butadienes with polymerizable compounds to form vulcanizable elastics; also such straight and mixed plastics can be modified by the use of plasticizers and other modifying agents.

In the drawing, which illustrates one embodiment of the invention:

Figure 1 represents a front plan view of a disc-shaped grinding wheel embodying the present invention.

Figure 2 is a sectional view taken along the line II-II of Figure 1.

The disc-shaped grinding wheel illustrated in Figures 1 and 2 consists of a bonded abrasive section 5 of any desired thickness and diameter, having a flat grinding face 6 and an opposite supporting face 7. The abrasive section 5 is composed of abrasive grain such as crystalline aluminum oxide or silicon carbide suitably bonded. The bond may be a vitrified ceramic material, or it may be a silicate, or a resin or a rubber compound. As a support to provide added strength during grinding and to provide a means for mounting, the abrasive section 5 is provided with a steel backing plate 8 rigidly and adhesively attached to the supporting face 7 of the abrasive section 5 by means of an intermediate layer of tie bond 9. To assist in the adherence of the tie bond 9 to the abrasive section 5 and metal plate 8, the supporting face 7 of the abrasive section and the inner face 10 of the steel plate are properly treated prior to assembly. The backing plate 8 is provided with a center arbor hole 11 and three bolt holes 12 for fastening the backed wheel to a mounting plate on the grinding machine. (The mounting plate is not shown.)

As the above description and drawing show, the final grinding wheel is composed of three main parts, namely, the abrasive section, the backing plate, and the tie bond uniting the abrasive section and the backing plate. In making such a wheel according to the present invention, the following steps are carried out.

(A) Preparation of the abrasive section for bonding.

(B) Preparation of the backing plate for bonding.

(C) Compounding and preparation of the tie bond.

(D) Uniting or combining the above three components.

A more detailed description of the various steps will be discussed now under the separate headings above named.

(A) Bonded abrasive sections can be united to metal supports by means of the tie bonds of the present invention irrespective of the type of bond used in the abrasive section; highly satisfactory results have been obtained with resin, vitrified, silicate and rubber-bonded abrasive sections. The abrasive sections are molded and formed by any one of the well known methods of making bonded abrasive shapes. The abrasive section of the specific wheel illustrated consists of a single disc of bonded abrasive material which can be any desired diameter and thickness. However, this continuous disc of abrasive may be replaced by a plurality of segments with the adjoining abrasive segments either suitably cemented at their adjacent faces or separated by clearance spaces so as to present in use a discontinuous grinding surface.

In preparing the bonded abrasive section for combination with the metal backing, the supporting face of the abrasive is cleaned with a wire brush and any loose dust or dirt removed by an air blast. On the clean, dry supporting face of the wheel, one or more thin coatings of cement are applied, and the wheel dried after each application of cement. After the last coating of cement has been applied and dried, the wheel is heated in an oven to a temperature of 250° F. A cement for applying to the supporting face of the wheel when polychloroprene tie bond material is employed can be made from vulcanizable compounded polychloroprene broken down to ce-

ment form in a solvent such as benzol or toluol. Two cements which have been found to be highly satisfactory for this purpose are ones sold on the market as Bostik M-117 and Bostik M-162.

(B) In the wheel illustrated, the backing plate is of  $\frac{1}{8}$ " mild steel cut the same diameter as the abrasive section. The backing plate does not necessarily have to be of a size to cover the entire back of the abrasive section and may be of a different material and thickness. It may also have other means of machine mounting than the centrally-located bolt holes of the depicted embodiment.

The steel backing plate is first properly cleaned to remove all oil and dirt. The plate surface for contact with the tie bond is then prepared to receive the cement and tie bond. This can be done by the use of an ordinary commercial pickling procedure followed by washing and drying, which, when used in connection with the present tie bonds, gives an entirely satisfactory surface for adhesion. After the plate has been prepared as above, it is given one or more coatings of a cement similar to that used on the supporting face of the abrasive section. After the cement has been dried, the plate is ready for use.

(C) The intermediate layer referred to herein as the tie bond consists of a layer of soft, pliable, resilient material in the form of a thin sheet approximately  $\frac{1}{16}$ "- $\frac{1}{8}$ " in thickness, although the thickness may vary somewhat from these figures. By selection of the proper thickness of this intermediate layer, the desired degree of resilience, i. e., resistance to mechanical shock, of the wheel can be closely controlled. Before use, the sheet of tie bond material is wiped clean and dry on both sides and a coating of cement such as that used on the backing plate and the abrasive section is applied to each side and allowed to dry.

(D) As a tie bond material, polychloroprene, especially when properly compounded, has been found to be highly effective in bonding the backing plate to the abrasive section. By the addition of a filler such as soft carbon black in sufficient quantities, a bond of extremely high strength has been obtained. Other fillers may be used to replace part or all of the soft carbon black, as, for example, channel black or mineral fillers such as blanc fixe, natural whiting, Dixie clay and the like, although soft carbon black is the preferred filler and produces the best results. Also, a part of the polychloroprene can be replaced by a natural rubber or a reclaimed rubber.

A tie bond material which is highly satisfactory for the present use is made of the following ingredients compounded and sheeted to the desired thickness on a roll mill.

|                               | Parts by weight |
|-------------------------------|-----------------|
| Polychloroprene               | 100             |
| Extra light calcined magnesia | 4               |
| Zinc oxide                    | 5               |
| Soft carbon black             | 200             |
| Cottonseed oil                | 5               |
| Sulfur                        | 1               |
| Phenyl-beta-naphthylamine     | 2               |

Polychloroprene, when it is properly compounded, as a fundamental or basic substance for tie bonds has been found to give very satisfactory results. It is a polymer of chloroprene, otherwise known as 2 chloro-1, 3-butadiene having the formula  $\text{CH}_2:\text{CHCl}:\text{CH}_2$ , and may be classified as being a halogen-substituted butadiene. A similar substance particularly effective as a tie bond is the copolymer of butadiene (divinyl) with acrylonitrile. Other compounds

which can be used instead of polychloroprene or butadiene-acrylonitrile copolymers are polymers of butadiene (divinyl), polyethylene sulphide and copolymers thereof, polymers and copolymers of vinyl chloride and vinyl acetate, copolymers of chloroprene and acrylonitrile, copolymers of butadiene (divinyl) with styrene, copolymers of butadiene (divinyl) with vinylidene chloride, copolymers of butadiene (divinyl) with methyl methacrylate, copolymers of butadiene (divinyl) with coumarone or isobrene, and copolymers of chloroprene with styrene, or methyl methacrylate. These are all substances having physical properties somewhat similar to polychloroprene. They are materials of high molecular weight and form tough, resilient, pliable solids which are vulcanizable. In vulcanized form, they withstand the heat evolved in dry grinding and are resistant to water and many hydrocarbon cooling agents used in wet grinding.

(D) After the tie bond has been prepared in sheet form and has been cut to the desired size for use with the backing plate and abrasive section, the three parts are assembled. The sheet of tie bond is placed upon the metal plate and smoothed down by running a roller over its surface to insure complete contact with the metal plate and to remove any air bubbles which may be trapped between the sheet and the metal. The abrasive section which has been kept in an oven at 250° F. is then removed and, while still hot, is placed on the tie bond sheet and metal plate. The assembly is centered on a mandrel to hold the parts in place during cure and the whole placed in a hot press. The tie bond is cured in the hot press under a pressure of 100-600 pounds per square inch at a temperature of 290-300° F. Thirty minutes is usually sufficient to adequately cure the wheel. For best results, the tie bond should be cured always under a pressure and temperature sufficient to cause it to extrude slightly at the edges from between the backing plate and the abrasive.

Abrasive wheels and discs of the present invention possess several beneficial properties which not only improve the general grinding characteristics of the wheels, but also extend their field of usefulness. For example, the present abrasive wheels have a long temperature range of serviceability extending from -30° to 300° Fahrenheit. Their retention of mechanical strength at high temperatures results in an increased factor of safety at normal operating speeds and also permits of higher speeds of operation when desirable. Also by reason of the high heat conductivity of the tie bond material, much of the heat generated in the abrasive section during use is quickly conducted through the tie bond layer to the metal support, where it is more easily dissipated by radiation, thus removing much of the danger of localized build-up of heat in the abrasive portions and thereby increasing the strength of the wheel.

Another important property of wheels of the present invention is their increased ability to absorb energy, a feature particularly important in grinding wheels which in the process of grinding are subjected to a repeated series of vibrations or shocks from contact with the work being ground. This ability to absorb energy is directly related to the ability to take up mechanical shock without damage to the wheel. This increased ability of the present wheels to absorb energy is coupled with a high rate of damping, so that, as a result, any vibrations from the shocks of

grinding are damped out quickly. As a result, the wheels are possessed of an increased strength and resistance to the shocks of grinding and can endure much more severe operating conditions.

5 In addition to accomplishing the objects and advantages previously set forth, the present invention offers numerous advantages which only become apparent in its use. For example, in preparing the backings for disc wheels and the like it has been found that with the present tie bonds it is no longer essential to sandblast the metal backing to obtain high adhesive strength, but a simple pickling treatment of the metal surfaces. This saves also the need of hammering the plates after the warping produced by sandblasting. Again, the parts after preparation do not require immediate assembling, but can be stored for later assembly at the convenience of the operator and availability of presses. Also, in 10 curing the present articles, the temperature and pressure of cure can be varied considerably without the danger of overcuring and its resultant loss of strength. These and other features lead to economies of manufacture not heretofore attainable.

15 It is not intended that the invention should be limited to the particular embodiment of wheel illustrated, as like objects and advantages are obtained in various other abrasive articles where it is necessary to secure bonded abrasive sections to metal or other rigid supporting or mounting means. For instance, similar disc wheels can be made in which the abrasive section is made of a plurality of individual segments properly spaced, 20 one from the other, to present a discontinuous grinding surface. Likewise, wheels for peripheral grinding may have supporting plates similarly secured to their flat side faces for added strength.

25 The present invention can also be used in the making of abrasive grinding rings or other shaped segments when it is desired to secure a metal support or mounting to the back or sides of the segment, or when, in the case of annular grinding shapes, it is desired to secure a metal ring to the internal or external circumferential surface of the ring away from the grinding surface as a reinforcement or means of mounting. Also 30 as an example of the application of the present invention, a number of large abrasive segments can be attached to a center ring of steel or other rigid material by means of a tie bond of vulcanizable synthetic elastic such as polychloroprene to form a pulp-wheel.

35 Likewise, small dental grinding stones such as cones and other shapes can be attached to steel mounting spindles by means of a vulcanizable tie bond such as set forth herein.

40 Having described the invention fully, it is desired to claim:

45 1. A bonded abrasive article comprising a bonded abrasive body, a rigid metal supporting means, and an intermediate cementing layer between said bonded abrasive body and said rigid metal supporting means adhesively uniting the two, said cementing layer comprising polychloroprene compounded with a substantial amount of a filler such as carbon black, and having an adhesive strength with respect to the bonded abrasive body and the rigid metal supporting means substantially in excess of that of the rubber bonds similarly employed.

50 2. A bonded abrasive article comprising a bonded abrasive body, a rigid metal supporting means, and an intermediate cementing layer be-

tween said bonded abrasive body and said rigid metal supporting means adhesively uniting the two, said cementing layer comprising a polymerized halogen-substituted butadiene compounded with a substantial amount of a filler such as carbon black, and having an adhesive strength with respect to the bonded abrasive body and the rigid metal supporting means substantially in excess of that of the rubber bonds similarly employed.

3. A bonded abrasive article comprising a bonded abrasive body, a rigid metal supporting means, and an intermediate cementing layer between said bonded abrasive body and said rigid metal supporting means adhesively uniting the two, said cementing layer comprising a member of the group consisting of polychloroprene, polychloroethylene, polydivinyl and polyethylenesulphide compounded with a substantial amount of a filler such as carbon black, and having an adhesive strength with respect to the bonded abrasive body and the rigid metal supporting means substantially in excess of that of the rubber bonds similarly employed.

4. A bonded abrasive article comprising a bonded abrasive body, a rigid metal supporting means, and an intermediate cementing layer between said bonded abrasive body and said rigid metal supporting means adhesively uniting the two, said cementing layer comprising a copolymer of polychloroprene and a copolymerizable resin compounded with a substantial amount of a filler such as carbon black, and having an adhesive strength with respect to the bonded abrasive body and the rigid metal supporting means substantially in excess of that of the rubber bonds similarly employed.

5. A bonded abrasive article comprising a bonded abrasive body, a rigid metal supporting means, and an intermediate cementing layer between said bonded abrasive body and said rigid metal supporting means adhesively uniting the two, said cementing layer comprising a copolymer of butadiene and a copolymerizable resin compounded with a substantial amount of a filler such as carbon black, and having an adhesive strength with respect to the bonded abrasive body and the rigid metal supporting means substantially in excess of that of the rubber bonds similarly employed.

6. A bonded abrasive article comprising a bonded abrasive body, a rigid metal supporting means, and an intermediate cementing layer between said bonded abrasive body and said rigid metal supporting means adhesively uniting the two, said cementing layer comprising a copolymer of butadiene and acrylonitrile compounded with a substantial amount of a filler such as carbon black, and having an adhesive strength with respect to the bonded abrasive body and the rigid metal supporting means substantially in excess of that of the rubber bonds similarly employed.

7. A bonded abrasive article comprising a bonded abrasive body, a rigid metal supporting means, and an intermediate cementing layer between said bonded abrasive body and said rigid metal supporting means adhesively uniting the two, said cementing layer comprising a member of the group consisting of polychloroprene, polychloroethylene, polydivinyl, and polyethylenesulphide modified by the copolymerization therewith of a copolymerizable resin com-

pounded with a substantial amount of a filler such as carbon black, and having an adhesive strength with respect to the bonded abrasive body and the rigid metal supporting means substantially in excess of that of the rubber bonds similarly employed.

8. A bonded abrasive article comprising a bonded abrasive body, a rigid metal supporting means, and an intermediate cementing layer between said bonded abrasive body and said rigid metal supporting means adhesively uniting the two, said cementing layer comprising a copolymer of butadiene and styrene compounded with a substantial amount of a filler such as carbon black, and having an adhesive strength with respect to the bonded abrasive body and the rigid metal supporting means substantially in excess of that of the rubber bonds similarly employed.

9. A bonded abrasive article comprising a bonded abrasive body, a rigid metal supporting means, and an intermediate cementing layer between said bonded abrasive body and said rigid metal supporting means adhesively uniting the two, said cementing layer comprising a copolymer of polychloroprene and a copolymerizable resin selected from the group consisting of acrylonitrile, styrene, methyl methacrylate, isobutylene, coumarone, indene, vinylidene chloride and chloromethacrylic ester compounded with a substantial amount of a filler such as carbon black and having an adhesive strength with respect to the bonded abrasive body and the rigid metal supporting means substantially in excess of that of the rubber bonds similarly employed.

10. A bonded abrasive article comprising a bonded abrasive body, a rigid metal supporting means, and an intermediate cementing layer between said bonded abrasive body and said rigid metal supporting means adhesively uniting the two, said cementing layer comprising a copolymer of butadiene and a copolymerizable resin selected from the group consisting of acrylonitrile, styrene, methyl methacrylate, isobutylene, coumarone, indene, vinylidene chloride, polyethylenesulphide, and chloromethacrylic ester, compounded with a substantial amount of a filler such as carbon black, and having an adhesive strength with respect to the bonded abrasive body and the rigid metal supporting means substantially in excess of that of the rubber bonds similarly employed.

11. A bonded abrasive article comprising a bonded abrasive body, a rigid metal supporting means, and an intermediate cementing layer between said bonded abrasive body and said rigid metal supporting means adhesively uniting the two, said cementing layer comprising a member of the group consisting of polychloroprene, polychloroethylene, polydivinyl, and polyethylenesulphide modified by the copolymerization therewith of a copolymerizable resin selected from the group consisting of acrylonitrile, styrene, methyl methacrylate, isobutylene, coumarone, indene, vinylidene chloride and chloromethacrylic ester, compounded with a substantial amount of a filler such as carbon black, and having an adhesive strength with respect to the bonded abrasive body and the rigid metal supporting means substantially in excess of that of the rubber bonds similarly employed.

GARRET VAN NIMWEGEN.